

## UNITED STATES PATENT OFFICE

2,245,155

## PROCESS FOR THE PRODUCTION OF SUBSTANTIALLY STABLE FUSED SALTPETER BATHS

Josef Martin Michel, Bitterfeld, Germany, assignor, by mesne assignments, to Walther H. Duisberg, New York, N. Y.

No Drawing. Application June 22, 1939, Serial No. 280,572. In Germany June 27, 1938

4 Claims. (Cl. 148—27)

This invention relates to a process for the production of substantially stable fused saltpeter baths, consisting substantially of sodium nitrate or potassium nitrate or mixtures thereof.

In the heat treatment of metals, especially light metals, use is frequently made of baths consisting substantially of fused saltpeter. In using such baths it has often been observed that the metals under treatment and also the metal containers containing the baths become corroded in course of time, leading to a local staining of the surface of the workpieces under treatment and the progressive formation of a highly inconvenient sludge consisting of solid reaction products. Recent investigations have shown that these phenomena are substantially caused by a progressive decomposition of the saltpeter baths which initially leads to the formation of nitrate, accompanied by liberation of oxygen; said nitrate subsequently decomposes to form free alkali. In order to prevent the corrosion of the workpieces in the bath, it has already been proposed to add chromates to the saltpeter baths. While such additions may succeed in suppressing the action of the decomposition products of the saltpeter baths on the metal undergoing treatment, they do not go to the root of the trouble since they do not prevent the decomposition, as such, of the baths.

It has now been ascertained that equilibria, dependent on the temperature, exist between saltpeter and its decomposition products, and that the progressive decomposition of saltpeter baths is caused by their tendency to attain the state of equilibrium at the actual working temperature of the bath. By incorporating at the outset in the (undecomposed) fused saltpeter bath, such amounts of the decomposition products as are required to establish the equilibrium at the bath temperature, the decomposition of the bath can thus be avoided.

The decomposition of the saltpeter proceeds in accordance with the following equations:



Accordingly, alkali metal nitrite and oxygen are formed in the first stage of the decomposition and then, through the decomposition of the alkali nitrite, free alkali and nitrogen trioxide. In presence of the oxygen simultaneously liberated, the free alkali reacts with a large number of the metals employed for the production of the fused baths or concerned in the heat treatment, with the formation of salts which are mostly insoluble in the melt and therefore settle down to

the bottom, as sludge, in the course of time. Since the saltpeter decomposition products thus continuously separate out from the bath, the decomposition practically never ceases.

Based on the foregoing discoveries, the present invention provides a process for the production of a substantially stable fused saltpeter bath, which comprises adding to fused saltpeter at least such an amount of alkali metal nitrite as will establish equilibrium between said saltpeter and said nitrite at the temperature at which said bath is intended to be used.

In carrying out the invention, it is preferable to add a slight excess of alkali metal nitrite over that corresponding to the equilibrium at the temperature at which the bath is intended to be used.

Since the addition of the alkali metal nitrite in accordance with the invention considerably lowers the liquidus point of the saline mixture, the fluidity of the bath at a given temperature, is increased. In the heat treatment of metals, such high fluidity of the saline bath is important, inasmuch as the losses of bath material, due to its adhesion to the workpieces on their removal from the bath, are correspondingly reduced. Moreover this reduction of the melting point of the saline baths occasionally enables them to be employed at temperatures at which baths consisting solely of saltpeter would already be solid.

In view of the relatively small quantities of nitrite required for stabilizing the saltpeter baths, the fact that the nitrite itself decomposes into nitrogen trioxide and alkali metal oxide, is of small practical consequence. This decomposition of the nitrite can however be counteracted by incorporating a small proportion of an alkali (such as alkali metal carbonate) in the bath. In order to prevent corrosion of the metals by the alkali, said alkali is preferably added in the form of neutral or slightly alkaline reacting salts of heavy-metal oxyacids of the kind known to have a passivating action on metals, such as alkali metal monochromates, alkali metal tungstates, alkali metal vanadates, and also the less soluble chromates of the alkaline-earth metals and zinc.

The required proportions of these passivating additions vary within a very narrow range, e. g. between about 0.1% and 1% in the case of alkali metal monochromates. In the case of alkaline-earth metal chromates or zinc chromate, the solubility of which in saltpeter melts at temperatures closely above the melting point of saltpeter is very slight, but strongly increases with

rising temperatures, it is always advisable to employ a slight excess, which can remain, as a harmless solid phase, in the melt.

The passivating effect on the metal surfaces in contact with the saline melt is of special importance in the employment, or treatment of iron and steel, because it prevents the formation of ferric oxide which has a catalytic decomposing action on salt peter.

The following table shows the amounts of sodium nitrite and nitrogen trioxide which are in equilibrium.

| Temperature, °C. | N <sub>2</sub> O <sub>3</sub> | NaNO <sub>2</sub> |
|------------------|-------------------------------|-------------------|
|                  | Percent                       | Percent           |
| 350.....         | 0.06                          | 0.09              |
| 400.....         | 0.13                          | 0.23              |
| 450.....         | 0.4                           | 0.72              |
| 500.....         | 1.3                           | 2.16              |
| 550.....         | 4.5                           | 8.11              |

The table shows and serves as an indication of the minimum proportions of alkali metal nitrite required for stabilizing the different salt peter baths at the various working temperatures specified.

I claim:

1. A process for the production of a fused salt peter bath substantially stable within a temperature range of between about 350 and 550° C., which comprises adding to said fused salt peter an amount of alkali metal nitrite approximately corresponding stoichiometrically to the amount of nitrite found in the salt peter bath at the operating temperature without the addition of alkali metal nitrite after equilibrium is reached. 35

2. A process for the production of a fused salt peter bath substantially stable within a temperature range of between about 350 and 550° C., which comprises adding to said fused salt peter an amount of alkali metal nitrite approximately corresponding stoichiometrically to the amount of nitrite found in the salt peter bath at the operating temperature without the addition of alkali metal nitrite after equilibrium is reached, and further a small proportion of an alkali.

3. A process for the production of a fused salt peter bath substantially stable within a temperature range of between about 350 and 550° C., which comprises adding to said fused salt peter an amount of alkali metal nitrite approximately corresponding stoichiometrically to the amount of nitrite found in the salt peter bath at the operating temperature without the addition of alkali metal nitrite after equilibrium is reached, and further a small proportion of at least one compound of the group consisting of the neutral and slightly alkaline reacting heavy metal oxy-acid salts having a passivating effect.

4. A process for the production of a fused salt peter bath substantially stable within a temperature range of between about 350 and 550° C., which comprises adding to said fused salt peter an amount of alkali metal nitrite approximately corresponding stoichiometrically to the amount of nitrite found in the salt peter bath at the operating temperature without the addition of alkali metal nitrite after equilibrium is reached, and further between 0.1 and 1% of an alkali metal chromate.

JOSEF MARTIN MICHEL.